

Oct. 7, 1941.

E. H. HOAG

2,258,507

FLOTATION PROCESS

Filed Aug. 27, 1940

3 Sheets-Sheet 1



Oct. 7, 1941.

E. H. HOAG

2,258,507

## FLOTATION PROCESS

Filed Aug. 27, 1940

3 Sheets-Sheet 2

A technical line drawing of a heat exchanger assembly. The drawing shows a central rectangular frame (10) containing two vertical heat exchanger units. Each unit has a U-shaped tube assembly (32) supported by vertical columns (25). The bottom section of the frame (15) contains two U-shaped tube assemblies (11) supported by vertical columns (14). A horizontal pipe (16) is connected to the top of the frame. A large vertical pipe (28) is connected to the right side of the frame. Various valves and fittings are shown throughout the system. The drawing is labeled with numbers 10, 12, 14, 15, 16, 17, 25, 28, 30, 32, 41, 41a, 41b, 45, 46, and 47.

INVENTOR  
EDWARD H. HOAG

Edmund P. Hayes

ATTORNEY

Oct. 7, 1941.

E. H. HOAG

2,258,507

## FLOTATION PROCESS

Filed Aug. 27, 1940

3 Sheets-Sheet 3

Fig. 5.



Rig. 6.



Fig. 7.



INVENTOR  
EDWARD H. HEAG

EDWARD H. HORN  
Edward H. Horn

*ATTORNEY*

## UNITED STATES PATENT OFFICE

2,258,507

## FLOTATION PROCESS

Edward Hammond Hoag, Los Angeles, Calif.

Application August 27, 1940, Serial No. 354,346

4 Claims. (Cl. 209—166)

This invention relates to the separation by mechanical, physical and chemical means of the valuable constituents of rocks, ores, minerals and chemical products based primarily on the difference in floatative properties of the content due to a combination of acts by which a definite and desirable electrical sign and charge is formed, or a modification of same, on the surface of said minerals or products.

An important object of the invention is to accelerate the time necessary to cause minerals to rise to the surface of pulp in the form of flotation froth and collect there as such into their respective classes and kinds.

Another important object is to provide a process that will activate or depress desirable or undesirable minerals in a flotation bath and separate them from each other by modifying the electrical sign and charge on the surface of said minerals.

Another object is to provide a flotation process in which the flotation bath is ionized by introducing therein direct current impulses to completely immersed electrodes interrupted for short intervals.

A further object is to cause an attraction of basic oxides, colloidal basic hydroxides and magnetizable minerals towards negative electrodes immersed in a flotation bath, to remove said minerals from the bath and to impede adsorption of colloidal basic hydroxides and hydrolysed silica.

A further object is to attract negative and positive suspensoids towards positive and negative electrodes respectively.

A further object is to impede film-forming minerals from depressing desirable minerals in the presence of activating reagents.

A further object is to flocculate colloidal mineral suspensions and prevent undesirable films from forming on desirable minerals.

A further object is to provide a new method for differential separation of minerals into commercial products.

A further object is to utilize the ions formed in a flotation bath or the ions released from reagents and conditioners by the introduction into said bath of direct current impulses interrupted for short intervals.

Further objects will hereinafter appear are

accomplished by means of the process described herein and illustrated in the accompanying drawings, in which:

Fig. 1 is a plan view of the apparatus, partly broken away and partly in section.

Fig. 2 is a central vertical section of the apparatus taken on line 2—2 of Fig. 1 looking in the direction indicated by the arrows therein.

Fig. 3 is a cross section of the apparatus taken on the line 3—3 of Fig. 2 looking in the direction indicated by the arrows thereon.

Fig. 4 is an end elevation of the apparatus.

Fig. 5 is a longitudinal section view of the ionization apparatus.

Fig. 6 is an electrical diagram of the circuit of the ionization apparatus.

Fig. 7 is an enlarged detail of the central portion of the agitation chamber of the apparatus illustrating the movement of the pulp during the operation of the apparatus.

Fig. 8 is a diagram of the electrical circuit for introducing into a flotation bath direct current impulses interrupted for short intervals by any well known interrupter 37.

Fig. 9 is an enlarged sectional plan in more detail of one of the air distributing pipes and adjacent electrodes connected in circuit with a source of electrical energy, showing direct current impulses introduced to electrodes completely immersed in a flotation bath 10, said currents interrupted for short intervals by the mechanical interrupter 37 used for breaking said circuits.

In the appended drawings I have illustrated an apparatus by means of which my improved process may be practiced efficiently.

In the drawings, 10 indicates the cell or tank of the apparatus, having upwardly and outwardly inclined side walls 11 and vertical end walls 12.

Centrally disposed and extending longitudinally of the cell 10 is a centrally disposed trough 13 through which the sands or heavy particles pass, and serves to bring the pulp into intimate contact with the impellers 14 mounted therein.

These impellers are of the usual form and are secured to the lower ends of hollow vertical shafts 15, their upper ends being provided with pulleys 16 belted to a suitable source of power as an electric motor 28 to operate the impellers,

air from a suitable source of power passing through the hollow shafts 15 into the pulp. The pulp is fed to the trough 13 through a conduit 17 where it is uniformly distributed by the impellers.

Arranged in the tank 10 and on each side of the impellers are vertically extending partitions 18 which define the agitation chamber 19, and disposed between the partitions 18 are a series of transversely disposed partitions 20 which divide the cell into a plurality of cells 21, in order that the pulp flowing therethrough may be retained in the agitation chamber 19 for time contact.

Positioned between the partitions 18 and the side walls of tank or cell 10 are longitudinal partitions 22 that form a plurality of quiescent chambers 23, and disposed in said chambers are perforated air distributing pipes 24 controlled by valves 25 by means of which the froth may be enriched during its agitation.

The rear wall of the tank 10 is provided with an opening 26 controlled by a weir gate 27 for regulating the level of the pulp in the tank.

Mounted one side of the tank 10 and preferably at its top portion is a driving motor 28 for operating the various devices employed in the apparatus as will be more fully set forth hereinafter.

Disposed on one of the top corners of the tank is a small electric generator M for generating direct current impulses for delivery to the pulp through the various electrodes disposed in the tank. Mounted on one of the upper corners of the tank and opposite to the generator M is a pressure blower 29 connected to an enlarged electrical air chamber 30 that leads to an ionization apparatus 31 which will be described with greater particularity hereinafter. The ionized air from apparatus 31 passes through a pipe line 32 to the various perforated pipes disposed in the chambers of the apparatus.

In addition to the ionizing apparatus for producing and injecting ions into the mineral pulp, an electrical apparatus is employed which preferably consists of a plurality of electrodes 33 disposed in the various chambers of the apparatus. These electrodes are arranged in positive and negative pairs, a pair to each chamber, their ends being secured in the end walls of the tank and insulated therefrom. These electrodes are preferably disposed at convenient heights near the perforated air pipes 24 and are completely immersed in the flotation bath.

The various pairs of electrodes are connected in circuit with the positive and negative terminals 34 and 35 of the generator M, an interrupter 37 of well-known type being interposed in the electrical circuit to break the direct current impulses for intervals of not less than one second.

The impellers, as well as all other operable mechanisms are actuated from the driving motor 28 through the agency of belts and pulleys in the usual well known manner.

Tailings are discharged through the opening 39 into launder 40, and for a very large capacity through 39a also, while the froth bearing the valuable concentrates overflows into the launders 41 secured to the side walls of the apparatus, the overflow lips 45 being adjustable to control the flow of froth thereto.

The enlarged detail of the lower portion of the tank as shown in Fig. 7 is to illustrate the passage of the pulp through the apparatus during beneficiation. Secured directly above the centrally disposed partition 20' and spaced therefrom to

form a passageway between the tank section A and B is a transversely disposed partition 20a designed to control the retention of froth in each tank section and the flow of pulp from the exit 5 toward the head in the agitation chamber of the apparatus during its treatment.

Pipe line 30a leading from the air pressure chamber 30 shown in Fig. 2, directs concentrates which overflow from section B of the tank to launder 41 and to 41a and how they may be returned to tank section A by a suitable air lift apparatus which includes 30a under low air pressure to enrich the lower grade concentrates from tank section B if such procedure is essential.

The source of current for operating the electrical elements mounted therein is delivered from an alternating current generator M' of any standard make that delivers an initial current varying from 110 to 440 volts, and this current can be "stepped up" to greater voltages, that is, from 5000 to 35,000 volts by means of the transformer 50 mounted in one end of the casing controlled by a rheostat 51, a rectifier R and a pair of two-way switches a and a' located on the switchboard.

In the drawings only a single electrode has been shown, but it is obvious that several may be employed depending upon the ionization required in the beneficiation of different classes of ores.

The electrode 55 here illustrated preferably consists of a central rod 56 formed of aluminum, its upper and lower ends passing through circular plugs 57, 58 formed of glass cement and secured to insulated plates 59 and 60 disposed within the ionization apparatus casing. Engaging the plugs 57 and 58 is a cylindrical glass tube 61, containing an intimate mixture of aluminum filings and carbon grains 62 tightly packed therein. Surrounding tube 61 and spaced therefrom as at 63 is an aluminum cylinder 64 provided with a plurality of perforations 65 for the release of ions formed by the electrode on their passage through the corona.

The operation of the ionization apparatus is as follows: The electrical current from the generator flows through a rheostat 51, from thence it is led to the primary winding of a transformer 50 by line wires 70 and 71. From the secondary windings 52 of the transformer it is conducted by line wires 53 and 54 to a synchronous rectifier R through line wires 53' and 54' to a pair of two-way switches a and a'. Negative ions are created and discharged through the perforated cylinder 64 of the electrode 55 by conducting the electrical current from transformer 50 through line wire 53 to synchronous rectifier R through line wire 53' and to a and thence through line wire 81 to electrode 55. Line wire 54 leads to synchronous rectifier R and through line wire 54' to switch a' through line wire 82 to perforated cylinder 64.

Positive ions are created in and discharged from cylinder 64 of the electrode 55 by connecting the current from transformer 50 through line wire 54 to synchronous rectifier R and through line 54' to switch a' through line wire 79 and switch a through line wire 81 to electrode 55. Line wire 53' leads to switch a through line wire 79 to switch a' through line wire 82 to 64.

According to the present invention a new method for the concentration of minerals by flotation is set forth by a series of acts all of which are combined or intimately related to each other to produce a novel result. They are as follows:

Introducing direct current impulses into a flota-

tion bath of known hydrogen ion concentration for a given temperature to completely immersed electrodes contained therein interrupted for intervals of not less than one second. The objective being to modify or change the electrical sign and charge on the surface of minerals; to allow some of the reagents or conditioners to return to their original status and structure after the flow of direct current impulses has been interrupted for short intervals; to accelerate the dissociation of molecules of reagents and conditioners as well as to furnish desirable additional ions to the bath for collecting or for conditioning purposes; to attract negative and positive mineral suspensoids towards the positive and negative electrodes respectively; and finally, to modify the hydrogen ion concentration of the flotation bath.

Introducing flotation reagents with the object of forming an insoluble film on the surface of minerals and to give said minerals-and-films a desirable electrical sign and charge.

Introducing conditioners for the purpose of modifying the electrical sign and charge on the surface of minerals as well as for modifying the pH value of the pulp.

Introducing ionized air to furnish positive or negative ions from the air for the air-oil-globule entity and for the mineral-and-film entity so as to have the desirable electrical sign and charge desirable for flotation of minerals.

The introduction of direct current impulses into the flotation bath to the immersed electrodes contained therein is a step which modifies or changes the electrical sign and charge on the surface of colloidal basic hydroxides, minerals in suspensions and film-forming minerals, and also serves to attract said minerals towards said electrodes until released by the interruption of the direct current impulses for short intervals. If said minerals are neutralized then their original electrical sign is changed or modified and therefore they do not exchange ions with other minerals or with reagents or chemicals in the same manner or intensity, as they do before the introduction of the flow of direct current impulses. Any change or modification of the hydrogen ion concentration of the flotation bath definitely changes or modifies the electrical sign and charge on the surface of minerals. If the pH value of the bath increases to a higher order of acidity or alkalinity then stabilization increases also to a certain degree. Some minerals adsorb others more intensely so it is obvious that different minerals in the same flotation bath are modified differently by any change or modification of the hydrogen ion concentration of the flotation bath. Some minerals can be destabilized during the interruption of direct current impulses or while they approach the isoelectric point. Minerals may be flocculated, depressed or precipitated by introducing into a flotation bath direct current impulses interrupted for short intervals when the electrical charge and sign are equal and opposite to that of the minerals.

Minerals in the depressed state submerge and join gangue materials in their exit from the bath.

The interruption of direct current impulses allows some reagents and conditioners to return to their original structure and status and to serve again in their original capacity for activating and depressing minerals.

When frothing oils are introduced into a flotation bath a film of oil is formed on the air-oil-globules taking a definite electrical sign from 75

said bath. That is, if the hydrogen ion concentration of the bath is acid then the film on the air-oil-globule takes a positive sign, and if the bath is alkaline then the oil film would take a negative sign. It is obvious then, that any change or modification in the pH value of the flotation bath means a change or modification in the electrical sign on the oil film of the air-oil-globule entity.

10 Flotation reagents when introduced into a flotation bath generally consist of molecules of the unsaturated type with free valences which in turn partly explains why they have such an intense attraction for minerals and also for the rapid exchange of their free ions with said minerals to form the insoluble film on their surfaces by adsorption.

15 Polar molecules such as CHO, COOH, and OH types change emulsoids to suspensoids by removal of the water film from the emulsions.

An electrical charge introduced into a flotation bath which is opposite and equivalent to the charge and sign on the mineral and film will neutralize it. This phenomena partly explains 20 how minerals can be depressed or precipitated; how the pH value of the flotation bath is modified, how minerals and reagents or negative or positive colloids and minerals of the opposite sign and charge are restrained from exchanging ions freely 25 with each other.

30 Flocculation is antecedent to flotation of minerals and the first step or importance before the physics of "wetting."

The stability of mineral suspensions represented by the magnitude of the electrical charge 35 and sign on their surface is modified by introducing direct current impulses into a flotation bath interrupted for short intervals, together with electrolytes, reagents and conditioners which give off ions of the opposite sign and charge to that of the minerals and solution. When minerals are suspended in a liquid medium I find negative reagents giving off large negative ions to negative minerals to increase their stability; and to positive 40 minerals to decrease their stability; and I also find, that positive reagents give large positive ions to increase the stability of positive minerals and to decrease the stability of negative minerals.

45 Negative or anionic reagents give off heavy negative ions presumably reacting on minerals suspended in a solution when dissociated by direct current impulses interrupted for short intervals as  $+H$  and  $-OH$  ions do in the presence of water, that is, they increase the negative and decrease the positive charge of electricity on the surface of minerals; or they decrease the pH value or increase the acidity or decrease the alkalinity of the solution; or they increase the stability of negative minerals and decrease the stability of positive minerals; or they increase flocculation of positive minerals and decrease flocculation of negative minerals.

50 Positive or cationic reagents under the above conditions give off heavy positive ions decreasing the negative charge and increasing the positive charge of electricity on the surface of minerals; or they increase the pH value or decrease the acidity or increase the alkalinity of the flotation bath; or they decrease the stability of negative 55 or increase the stability of positive minerals; or they decrease flocculation of positive or increase flocculation of negative minerals.

55 The pH value of a flotation bath is changed or modified by introducing direct current impulses to electrodes immersed therein and interrupted

for short intervals if said bath contains reagents or conditioners, by accelerating the dissociation of its molecules or by supplying desirable additional ions which are introduced therein. That is, negative reagents and conditioners will give off negative ions and the pH value of the solution will decrease or its acidity will increase while positive reagents and conditioners will give off positive ions and the pH value of the solution will increase or its alkalinity increases.

In view of the above the process is subordinate to changes or modifications of the sign and charge on the surface of minerals caused by introducing direct current impulses to a flotation bath to completely immersed electrodes contained therein and then interrupting the impulses for short intervals of not less than one second as referred to heretofore in combination with the other steps in the process, by which minerals are activated or depressed and the pH value of the pulp solution modified accordingly.

The process is also subordinate to the modified sign and charge on the surface of minerals caused by removing film-forming minerals from a flotation bath in order that said minerals cannot exchange their ions freely with undesirable minerals to activate them. For example, if a flotation bath contains colloidal basic hydroxides as suspensoids they will exchange ions freely with hydrolysed silica in the presence of positive conditioners and negative reagents in an alkaline circuit, by adsorption. If it is desirable to depress silica, then the colloidal basic hydroxides should be removed from the bath by attracting them towards the immersed negative electrodes and in this manner to deactivate the siliceous materials by suppressing the free exchange of ions between said colloids and the hydrolysed silica.

Direct current impulses introduced into a flotation bath and interrupted for short intervals of not less than one second in combination with the other steps in the process, assists in precipitating, neutralizing, flocculating or destabilizing minerals when they are in a fine state of suspension by restraining them from depressing desirable minerals in said bath, that is, if the electrical charge and sign is equivalent and opposite to the charge and sign on the mineral.

When minerals are in a fine state of suspension or in a colloidal condition in a flotation bath, they are known to be electrically charged with a positive or negative sign. Such minerals that are attracted towards positive electrodes during the flow of direct current impulses are classed as negative minerals and a few of them included in this class which are found in the following example to illustrate the process are gold, silver, arsenious sulfides, cupric sulfide, sulfides of iron, antimony, arsenic, lead and copper. Minerals in suspension which are attracted towards the negative electrodes during the flow of direct current impulses are classed as positive minerals and included in this class are hydroxides of aluminum, ferric, copper and others.

The phenomena referred to above is illustrated by the following example:

The ore under consideration consists of pyrite, chalcopyrite, sphalerite, galena, associated with gold and silver minerals in a matrix of quartz, calcite, clays, and mica. It also contains colloidal basic hydroxides of iron and alumina, magnetite and hematite. It is a mixture of sulfides and non-sulfides containing fine grained minerals in suspension and containing minerals

charged electrically due to grinding operations in a mill, and finally, oxides of the above metals formed by nature.

The tails consist of siliceous materials, calcite, aluminum compounds, oxides, positive and negative colloids, oxides of iron, alumina and some of the valuable constituents in the ore as suspensoids, clays, micas, together with small amounts of sulfides of the metallic content and "rusty" gold.

10 The process consists of a series of acts by which materials are transformed into a new state, that is, physically due to the changes or modifications of their electrical charge and sign on the surface of minerals, or chemically by metathetical exchanges between molecules or by adsorption, and said acts are related to each other and necessary for the improved flotation of minerals.

15 The procedure to practice the invention for the above ore is as follows:

First introduce into a flotation bath direct current impulses of 220 volts and 1.5 amperes to completely immersed electrodes contained therein for approximately 3 seconds. The impulses are interrupted for intervals of 3 seconds by a mechanical interruptor which breaks the current for desirable intervals.

20 Secondly, the hydrogen ion concentration of the flotation bath is determined in terms of acidity or alkalinity for a given temperature such as the system taught by "La Motte Chemical Company" or by the "Beckman pH Meter" or "Potentiometer."

25 Thirdly, ionized air is introduced into the flotation bath consisting of either positive or negative ions and indicated by the pH value of the bath. Positive ions from the air are introduced into the bath when the pH value is above 7.0 and negative ions when the pH value of the bath is below 7.0.

Fourthly, flotation reagents and conditioners are introduced into the bath and consist of the types which give off heavy negative or positive ions.

30 Fifthly, the ore consists of both negative and positive minerals, that is, in the above example the negative minerals are chalcopyrite, galena, pyrite, quartz, calcite, and mica and the positive minerals are the colloidal basic hydroxides, basic oxides and other oxidized ores.

Sixthly, the film of oil on the air-oil-globule entity takes either a negative or positive electrical sign on its surface according to the pH value of the flotation bath. That is, the film of oil is positive when the flotation bath is acidic or the film is negative when the bath is alkaline.

Seventhly, conditioners introduced into the flotation bath have the important role of modifying the hydrogen ion concentration of said bath by giving off heavy negative or positive ions and exchanging their ions freely with minerals and reagents.

Eighthly, the insoluble film which is formed on the surface of minerals is due to the free exchange of ions between minerals and flotation reagents and conditioners, by adsorption.

Ninthly, the electrical charge on the surface of minerals is modified by introducing ions into the flotation bath of direct current impulses interrupted for short intervals in combination with the other steps in the process such as introducing ionized air, electrolytes and flotation reagents.

The changes in the electrical sign on the surface of minerals due to the free exchange of ions are illustrated in the following example:

Electrical sign  
of the effective ion

In this example, the gold content, lead and silver sulfides and chalcopyrite are the minerals desirable to float as a lead concentrate, while pyrite, sphalerite, quartz, calcite and mica are depressed. The zinc minerals are floated in a separate zinc cell as zinc concentrates.

First, direct current impulses of 220 volts and 1.5 amperes are introduced into the flotation bath to the immersed electrodes contained therein for 3 seconds and then interrupted for three seconds. The object of this is to cause positive colloidal basic hydroxides to be attracted towards the negative electrodes to impede the free exchange of ions between said colloids and siliceous materials and in this manner to avoid activating negative silica by adsorption. It is also for the purpose of modifying the pH value of the bath, for accelerating the release of the ions from reagents and conditioners, for attracting negative colloids towards positive electrodes, for the return of some of the reagents to their original status and structure after interruption of current impulses, and in the present case to assist in making the flotation bath alkaline so that its hydrogen ion concentration is 8.2.

Secondly, the negative minerals are chalcopyrite and galena. The electrical sign of the effective ion is

Thirdly, the kind of conditioners introduced into the flotation bath are neutral to chalcopyrite and galena but depress pyrite and sphalerite. These conditioners for example are zinc sulphate (1.90 lbs. per ton) and sodium cyanide (0.3 lb. per ton). The electrical sign of the effective ion is

Fourthly, the conditioner which gives off positive ions is soda ash (1.0 lb. per ton for this ore) by exchanging them freely with galena and chalcopyrite. The electrical sign of the effective ion is

Fifthly, the negative reagent introduced into the flotation bath which furnishes negative ions is potassium xanthate (0.06 lb. per ton of ore). It exchanges ions freely with the minerals to form the insoluble film on their surfaces by adsorption. The electrical sign of the effective ion is

Sixthly, positive ions from ionized air are introduced into the flotation bath for "wetting" purposes, that is, so that the film and mineral is surrounded by air and is water repellent. The electrical sign of the effective ion is

Seventhly, the frother cresylic acid (0.04 lb. per ton) furnishes the negative ions for the film of oil surrounding the air-oil-globule entity. The electrical sign of the effective ion is

Eighthly, positive ions introduced into the bath from the air completes the process for flotation of the mineral-and-film entity and the air-oil-globule entity. The electrical sign of the effective ion is

In the above example the flotation bath was alkaline due to the introduction of direct current impulses interrupted for short intervals together with positive conditioners. The reagents used were of the negative type, the ions from the air were of the positive type, the conditioners furnished positive ions and the minerals present that were floated were of the negative type. The positive colloids were detained in the pulp and the negative suspensoids were flocculated.

If the order of the positive and negative electrical signs of the effective ions were interchanged in the example as illustrated, then flotation of the minerals would not be economically improved. For example, if negative ions from the air were introduced into the flotation bath instead of positive ions, or if the pulp was acidic instead of alkaline, or if the minerals were of the positive type instead of negative, or if direct current impulses were suspended, then, the process would not be economically improved.

The direct current impulses interrupted for short intervals in combination with the other 75

steps in the process when introduced into the flotation bath function in the general scheme of the process by accelerating the release of the effective ions of the reagents and conditioners, by furnishing desirable additional ions to the pulp to modify the pH value of the flotation bath, by attracting positive colloidal basic hydroxides towards the negative electrodes which are completely immersed therein to prevent said colloids from adsorbing siliceous materials, by attracting negative and positive colloidal suspensions towards positive and negative electrodes to flocculate them respectively by neutralizing dispersed particles, by precipitating depressed minerals and removing them together with colloidal basic hydroxides and film-forming minerals from the bath, by allowing some reagents to return to their original status and structure for further use in a continuous cycle of beneficiation, by removing undesirable suspensoids after neutralization of charge on their surfaces to avoid adsorption of desirable minerals, and by providing for a new arrangement of molecular structure for some of the reagents and minerals with their changed electrical sign and charge of improved flotation purposes.

Table 1

30 Shows the results of introducing into a flotation bath direct current impulses to electrodes completely immersed therein of adequate voltage and amperage to furnish desirable additional ions to said bath interrupted for intervals of not less than one second and introducing into the bath ionized air, flotation reagents, conditioners and emulsifiers for activation or depression of minerals contained therein.

| Positive | 35 | Product              | Weight | Assays per ton |         |         |         |         |         |
|----------|----|----------------------|--------|----------------|---------|---------|---------|---------|---------|
|          |    |                      |        | Au             | Ag      | Pb      | Zn      | Cu      | Fe      |
| Negative | 40 | Percent              | Ounces | Ounces         | Percent | Percent | Percent | Percent | Percent |
|          |    | Calc. head           | 100.00 | 0.04           | 19.00   | 5.70    | 6.50    | 0.80    | 5.60    |
|          |    | Lead conc.           | 11.00  | 0.335          | 162.36  | 51.10   | 4.88    | 6.90    | 3.58    |
|          |    | Zinc conc.           | 15.00  | 0.013          | 3.77    | 0.20    | 37.30   | 0.20    | 13.28   |
|          |    | Tails                | 75.00  | 0.0016         | 0.765   | 0.013   | 0.49    | 0.015   | 4.288   |
| Positive | 45 | Distribution percent |        |                |         |         |         |         |         |
|          |    | Calc. head           | 100.00 | 100.00         | 100.00  | 100.00  | 100.00  | 100.00  |         |
| Negative | 45 | Lead conc.           | 92.20  | 94.00          | 98.51   | 8.26    | 94.91   | 7.04    |         |
|          |    | Zinc conc.           | 4.85   | 2.98           | 0.49    | 86.08   | 3.39    | 35.52   |         |
|          |    | Tails                | 2.95   | 3.02           | 1.00    | 5.65    | 1.70    | 57.44   |         |
| Positive | 50 | Assays per ton       |        |                |         |         |         |         |         |
|          |    | Au                   | Ag     | Pb             | Zn      | Cu      | Fe      |         |         |
|          |    | Percent              | Ounces | Ounces         | Percent | Percent | Percent |         |         |
|          |    | Calc. head           | 100.00 | 0.04           | 19.00   | 5.70    | 6.50    | 0.80    | 5.60    |
|          |    | Lead conc.           | 13.00  | 0.28           | 131.49  | 35.00   | 8.34    | 3.92    | 2.36    |
|          |    | Zinc conc.           | 16.00  | 0.014          | 7.112   | 5.06    | 32.24   | 1.60    | 16.93   |
|          |    | Tails                | 71.00  | 0.002          | 1.03    | 0.48    | 0.37    | 0.048   | 3.635   |
| Positive | 50 | Distribution percent |        |                |         |         |         |         |         |
|          |    | Calc. head           | 100.00 | 100.00         | 100.00  | 100.00  | 100.00  | 100.00  |         |
|          |    | Lead conc.           | 90.88  | 89.97          | 79.83   | 16.66   | 63.79   | 5.51    |         |
|          |    | Zinc conc.           | 5.63   | 5.99           | 14.20   | 78.36   | 32.00   | 48.40   |         |
|          |    | Tails                | 3.49   | 4.04           | 5.97    | 3.93    | 4.21    | 46.09   |         |

Table 2

55 Shows results after introducing into a flotation bath ionized air, flotation reagents and emulsifiers in pounds per ton the same as per Table No. 1, but without introducing into said bath direct current impulses to immersed electrodes interrupted for short intervals as per Table No. 1.

| Product | Weight | Assays per ton       |        |        |         |         |         |
|---------|--------|----------------------|--------|--------|---------|---------|---------|
|         |        | Au                   | Ag     | Pb     | Zn      | Cu      | Fe      |
|         |        | Percent              | Ounces | Ounces | Percent | Percent | Percent |
|         |        | Calc. head           | 100.00 | 0.04   | 19.00   | 5.70    | 6.50    |
|         |        | Lead conc.           | 13.00  | 0.28   | 131.49  | 35.00   | 8.34    |
|         |        | Zinc conc.           | 16.00  | 0.014  | 7.112   | 5.06    | 32.24   |
|         |        | Tails                | 71.00  | 0.002  | 1.03    | 0.48    | 0.37    |
| Product | Weight | Distribution percent |        |        |         |         |         |
|         |        | Calc. head           | 100.00 | 100.00 | 100.00  | 100.00  | 100.00  |
|         |        | Lead conc.           | 90.88  | 89.97  | 79.83   | 16.66   | 63.79   |
|         |        | Zinc conc.           | 5.63   | 5.99   | 14.20   | 78.36   | 32.00   |
|         |        | Tails                | 3.49   | 4.04   | 5.97    | 3.93    | 4.21    |

The pH value of the flotation bath is 7.5.

Reagents and conditioners used in Tables No. 1  
and No. 2

| Reagents used           | Conditioners | Rougher | Cleaner | Conditioners | Rougher | Cleaner | Scavengers |
|-------------------------|--------------|---------|---------|--------------|---------|---------|------------|
| Zinc sulphate.....      | 1.00         |         |         |              |         |         |            |
| Sodium cyanide.....     | 0.30         |         | 0.10    |              |         |         |            |
| Soda ash.....           | 1.00         |         |         | 1.50         |         |         |            |
| Copper sulphate.....    |              |         |         |              |         |         |            |
| Sodium silicate.....    |              |         | 0.15    |              | 0.10    | 0.15    |            |
| Pot. xanthate.....      |              | 0.06    |         |              | 0.10    |         | 0.04       |
| A. Cy. Re. No. 242..... |              | 0.04    |         |              | 0.10    |         | 0.04       |
| A. Cy. Re. No. 238..... |              | 0.04    |         |              | 0.04    |         | 0.15       |
| Sodium oleate.....      |              |         |         |              |         |         | 0.08       |
| Cresylic acid.....      |              | 0.04    |         |              |         |         |            |
| Amyl xanthate.....      |              | 0.04    |         |              | 0.04    |         |            |

Re. No. 242 is neutralized Aerofloat Flotation Reagent 31 sold by A. Cy. Co.  
Re. No. 238 is a dry Aerofloat Flotation Reagent of the dithiophosphorus class sold by A. Cy. Co.

The tails in the weight percent column of Table No. 1 shows that silica and calcite (negative minerals) are higher in content than in Table No. 2, proving that direct current impulses interrupted for intervals not less than one second materially aid in depressing undesirable minerals as well as flocculating negative mineral suspensoids. Likewise, it shows that the percentage of undesirable dispersed particles which have been depressed after neutralization increases.

Table No. 1 shows that iron and aluminum basic oxides and colloidal basic hydroxides are higher in content in the tails than in Table No. 2, indicating that direct current impulses flowing to the electrodes immersed in the flotation bath attract said minerals towards the electrodes and assist in reducing adsorption and activation of siliceous materials by said colloidal basic hydroxides.

Table No. 1 shows an improvement in the percent extraction of flotation of gold, silver, lead and copper in the lead concentrate and zinc in the zinc concentrate proving that it is an improved differential method for flotation of these minerals.

The tails of Table No. 2 show an increase in percentage of colloids which are floated with the zinc concentrates over the results in Table No. 1, indicating that direct current impulses interrupted for short intervals improves the grade of zinc concentrate.

Table No. 1 shows improved higher values for gold, silver, lead and copper in the lead concentrates than in Table No. 2 indicating that undesirable film-forming minerals are detained from forming films on desirable minerals in the bath and also, restrain film-forming minerals from depressing desirable minerals.

The results of Table No. 1 show a decided improvement in extraction and grade of minerals over the results in Table No. 2 and this difference is assigned to the novel steps in the combination process. These results indicate that colloidal basic hydroxides (iron hydroxides) are restrained from activating undesirable minerals such as silica; that film-forming minerals (aluminum oxides) are restrained from depressing desirable minerals such as the sulfides of silver, lead, copper and zinc; that basic iron oxides (hematite) are removed from the bath before they form films with the oleates on negative minerals such as on calcite and silica; that negative and positive suspensoids as well as the reagents, conditioners and emulsifiers modify the pH value of the bath, and finally, it illustrates that the electrical sign and potential on the surface of minerals is modified by the films formed on said minerals whether due to electrostatic charges,

20

or to metathesis, or to anchored ions or to chemical reactions between metal ions from oxidized surfaces and organic acid radicals of the collecting agents.

25

The tables prove that the steps in the process to obtain these results contribute to modify the pH value of the flotation bath, (Table No. 1 shows a pH value 8.2 and Table No. 2 shows a pH value 7.5), and obviously changes the electrical sign and potential of the air-oil-bubble entity and the mineral-and-film entity.

30

The ions furnished by zinc sulphate and sodium cyanide are neutral to galena and chalcopyrite but depress sphalerite and pyrite. The ions furnished by soda ash are positive and serve to condition the lead and copper minerals but depress iron more than zinc in an alkaline bath. The ions furnished by copper sulphate are of the negative type and for the purpose of activating zinc minerals. The ions of cresylic acid are negative and furnish the electrical sign of the oil film on the air-oil-globule entity. The ions furnished by sodium oleate are positive and activate oxides of minerals.

35

The introduction into the flotation bath of direct current impulses of 220 volts and 1.5 amperes interrupted for short intervals of 3 seconds accelerated the release of dissociated ions of flotation reagents and conditioners in said bath, modified the hydrogen ion concentration of the bath and furnished positive and negative ions to the bath.

40

Positive ions from the air were introduced into the flotation bath because said bath was predetermined as alkaline.

45

The mineral content of the bath furnished both negative and positive ions.

50

The final charge and sign of the ions on the surface of the mineral-and-film entity and the final charge and sign on the air-oil-bubble entity determined the status of the mineral for activation or depression.

55

Application of the process to any ore under all conditions is illustrated further as follows:

60

First, it is necessary to determine the hydrogen ion concentration of the pulp and the nature of the minerals in the pulp desirable to float, that is, whether they are of the negative or positive type.

65

Secondly, introduce direct current impulses into the flotation bath to completely immersed electrodes contained therein in adequate voltage and amperage to electrolyse the solution or to supply desirable additional ions, or for the purpose of orienting or grouping minerals, or to attract colloids, basic hydroxides or magnetizable minerals towards the electrodes, or to flocculate,

70

75

destabilize or precipitate minerals, or finally, to modify the pH value of the flotation bath.

If the pH value of the bath is found to be less than 7.0 or to be acidic, then negative ions from the air are introduced into the bath. The oil film surrounding the air-oil-globule has a positive electrical sign and the film of air for "wetting" purposes surrounding the mineral-and-film entity has a negative electrical sign. At this point indicated by a mark X for convenience there are two conditions presented, that is, whether it is desirable to float negative or positive minerals.

#### Case I

If it is elected to float positive minerals, then continuing with the process from X, I introduce positive reagents into the flotation bath, then negative conditioners. The desirable mineral has a positive electrical sign. A summary of Case I is as follows:

1. Positive minerals are floated from the flotation bath.

2. Negative conditioners are introduced to modify the pH value of the pulp.

3. Positive reagents are introduced to furnish positive ions and for forming the insoluble film on the surface of minerals with its electrical sign.

4. Negative ions from the air are introduced for "wetting" purposes, that is, to make the mineral-and-film water repellent.

5. Positive oil films are furnished by the frother and for the film on air-oil-globules.

6. Negative ions from the air are introduced to complete the process for forming the air-oil-globule and mineral-and-film entities with their electrical signs and charges for flotation of minerals.

The pH value of the flotation bath is below 7.0 and acidic.

The voltage and amperage of the direct current impulses interrupted for short intervals is adequate to dissociate the molecules of the solution in the bath or is introduced into the pulp to accelerate the release of ions from reagents or to modify the pH value of the flotation bath, or to furnish desirable additional ions to the bath, or to attract negative or positive suspensoids towards positive or negative electrodes respectively.

#### Case II

If it is desirable to use negative reagents in the above Case II instead of positive reagents, then it will be necessary to use positive conditioners, while the remaining steps in the process are as follows; that is, I introduce into the pulp negative ions from the air, positive conditioners and negative reagents for positive minerals.

The pH value of the flotation bath is below 7.0 and acidic.

The direct current impulses are introduced into the bath for similar reasons as indicated in Case I.

#### Case III

If it is elected to float negative minerals instead of positive minerals, then continuing with the process from the mark X, I introduce positive reagents into the flotation bath to form the insoluble film on the surface of minerals. The desirable mineral has a negative electrical sign.

Under this example, when the bath is acidic or its pH value is below 7.0 and direct current impulses have been introduced into the flotation bath and interrupted for intervals of not less than one second, the following summary exists:

1. Negative minerals are floated from the flotation bath.

2. Positive reagents furnish the positive electrical sign and for forming the insoluble film on the surface of the minerals.

3. Negative ions from the air are for "wetting" purposes.

4. Positive oil films are furnished by the frother and for the air-oil-globules.

5. Negative ions from the air are introduced to complete the process for forming the air-oil-globules entity and the mineral-and-film entity.

The pH value of the flotation bath is below 7.0 and acidic.

The voltage and amperage of the direct current impulses interrupted for short intervals is adequate to dissociate the molecules of the solution in the bath or is introduced into the pulp to accelerate the release of ions of reagents or

20 to modify the pH value of the flotation bath, or to furnish desirable additional ions to the bath, or to attract negative or positive suspensoids towards positive or negative electrodes respectively.

25

The voltage and amperage of the direct current impulses interrupted for short intervals is adequate to dissociate the molecules of the solution in the bath or is introduced into the pulp to accelerate the release of ions of reagents or

30 to modify the pH value of the flotation bath, or to furnish desirable additional ions to the bath, or to attract negative or positive suspensoids towards positive or negative electrodes respectively.

35

The pH value of the bath is found to be below 7.0 and acidic.

The direct current impulses are introduced into

the bath for similar reasons as indicated for Case III.

#### Case IV

If it is desirable to use negative reagents instead of positive reagents as in Case III then the conditioners introduced into the bath must be of the type which furnish large positive ions while all of the remaining steps in the process are as follows, i. e., I introduce into the pulp positive conditioners, negative reagents and negative ions from the air, for negative minerals.

The pH value of the bath is found to be below 7.0 and acidic.

The direct current impulses are introduced into

the bath for similar reasons as indicated for Case III.

#### Case V

If the pH value of the pulp is found to be greater than 7.0 or to be alkaline I introduce positive ions from the air into the flotation bath. The oil film surrounding the air-oil-globule is negative and the film of the air for "wetting" purposes on the insoluble film-and-mineral is positive.

At this point marked X' for convenience there are two conditions to consider that is, whether it is desirable to float negative or positive minerals.

If it is elected to float negative minerals then, continuing with the process from the point marked X', I introduce into the flotation bath negative reagents to form insoluble films on their surfaces. I introduce positive conditioners to exchange ions freely with desirable minerals but less so with undesirable minerals. Lastly, the desirable minerals to float have a negative electrical sign.

Under this example when the bath is alkaline and direct current impulses are introduced into the bath and interrupted for intervals of not less than one second, the following conditions exist:

65 1. Negative minerals are floated from the flotation bath.

2. Positive conditioners exchange ions freely with some of the minerals for conditioning purposes.

3. Negative reagents furnish negative ions freely with desirable minerals and for forming the insoluble film on the surface of minerals.

4. Positive ions from the air are introduced for "wetting" purposes.

75

5. Negative oil films are furnished by frother and for the film on the air-oil-globules.

6. Positive ions from the air are introduced into the bath to complete the process.

The pH value of the pulp is above 7.0 or alkaline.

The voltage and the amperage of the direct current impulses interrupted for short intervals is adequate to dissociate the molecules of the solution in the bath, or is introduced into the pulp to accelerate the release of ions of reagents or to modify the pH value of the flotation bath, or to furnish desirable additional ions to the bath, or to attract negative or positive suspensoids towards positive or negative electrodes respectively. 15

#### Case VI

If it is desirable to use positive reagents instead of negative reagents as in Case V then, the conditioners introduced into the bath must be of the type which furnish large negative ions while all of the other conditions of Case V are similar, that is, I introduce into the pulp negative conditioners, positive reagents and positive ions from the air for negative minerals.

#### Case VII

If it is elected to float positive minerals then continuing with the process from X', I introduce negative reagents into the flotation bath to exchange ions freely with desirable minerals and to form insoluble films on their surfaces. Finally, the desirable mineral to float has a negative electrical sign.

Under this example when the bath is alkaline and direct current impulses are introduced to the bath and interrupted for intervals of not less than one second, the following conditions exist:

1. Positive minerals are floated from the flotation bath.

2. Negative reagents furnish negative ions freely to exchange with said minerals and for forming insoluble films on the surface of positive minerals.

3. Positive ions from the air are introduced for "wetting" purposes.

4. Negative oil films are furnished by frothers and for the film on the air-oil-globule entity.

5. Positive ions from the air are introduced into the bath to complete the process for forming the mineral-and-film entity and the air-oil-globule entity.

The pH value of the pulp is above 7.0 or alkaline.

The voltage and amperage of the direct current impulses interrupted for short intervals is adequate to dissociate molecules of the solution in the bath, or is introduced into the pulp to accelerate the release of ions of reagents or to modify the pH value of the flotation bath, or to furnish desirable additional ions to the bath, or to attract negative or positive suspensoids towards positive or negative electrodes respectively.

#### Case VIII

If it is desirable to use positive reagents instead of negative reagents as in Case VII then the conditioners introduced into the bath must be of the type which furnish negative ions while the other conditions of Case VII are similar, that 70

is, I introduce into the pulp positive reagents, negative conditioners and positive ions from the air for positive minerals.

The pH value of the pulp is above 7.0 or alkaline.

The direct current impulses are introduced into the bath for similar reasons as indicated for Case VII.

The conditioners and reagents introduced into the flotation bath should be of such a nature that they are qualified to exchange ions freely with said minerals but not necessarily in the same manner with all minerals. Therefore, it is possible to depress some minerals while activating others in the same bath. The process is found to be applicable to any ore whether it is of the sulfide or non-sulfide type. The free exchange of ions of positive and negative minerals, positive and negative ions of electrolytes, emulsifiers and reagents, the positive and negative ions from ionized air released by the introduction of direct current impulses interrupted for intervals for not less than one second for modifying the hydrogen ion concentration of the flotation bath, are the steps in the process by which the broad concept and adaptability of the process to any class of ore is clearly indicated.

If the above procedure as outlined is not closely adhered to, then, flotation results will not be improved.

The eight cases cited show the acidity and alkalinity of the flotation bath and indicate at once what the electrical sign is on the surface of the oil-film of the air-oil-entity. They also indicate whether to introduce negative or positive ions from the air into the bath. That is, if the pulp is acid introduce negative ions from the air and if alkaline introduce positive ions from the air into said bath. The positive and negative reagents and conditioners introduced into the bath give off positive and negative ions which can be interchanged as cited. If the steps which the process consists of are not followed as set forth in these eight cases and direct current impulses are suspended from being introduced into the bath, then, flotation of the minerals will not be improved.

I claim:

1. A froth flotation process for minerals which comprises subjecting a pulp of the ore to be separated to agitation and aeration in the presence of a collector for the desired mineral and intermittently passing a unidirectional electric current through the bath below the surface, the intervals of the current flow and intervals between current flow being substantially 1 to 3 seconds duration.

2. The process as claimed in claim 1 in which aeration is accomplished with ionized air.

3. A froth flotation process as called for in claim 1 wherein the ore treated includes siliceous minerals and colloidal basic hydroxides.

4. A froth process as claimed in claim 1 in which the ore contains negatively charged minerals and positively charged colloids and suspensoids, and wherein the aeration is accomplished with ionized air, whereby the exchange of ions between the minerals and colloids is prevented.

E. H. HOAG.